

## UNITED STATES PATENT OFFICE.

OTTO KRESS, OF APPLETON, WISCONSIN, ASSIGNOR TO AMERICAN LAKES PAPER COMPANY, OF CHICAGO, ILLINOIS, A CORPORATION OF DELAWARE.

## METHOD OF BLEACHING PAPER PULP.

No Drawing.

Application filed December 24, 1925. Serial No. 77,622.

The invention relates to the bleaching of chemical wood pulp and more particularly to the bleaching of sulphate or so called "kraft" pulp. With the ordinary methods 5 of bleaching by means of bleaching powder (calcium hypochlorite) sulphate or "kraft" pulp can be bleached to a yellow color without serious loss in yield or strength, but it is impractical to bring this pulp to a satisfactory white color through the use of 10 bleaching powder or like oxidizing chlorine bleaching agents without decidedly impairing its characteristic strength and toughness and without materially reducing the yield. 15 The present improvement seeks to provide a method of bleaching chemical wood pulp and more particularly sulphate or "kraft" pulp to produce a satisfactory light color without serious deterioration either in the yield or in the strength of the pulp. 20

The present improvement consists in first bleaching the pulp in the ordinary way with a chlorine bleaching agent, preferably bleaching powder, the amount of such agent 25 being preferably such that the maximum bleaching effect will be produced without however effecting a substantial or serious decrease in the strength or in the yield of the pulp. The partially bleached pulp is then 30 subjected to the action of a reducing bleaching agent containing an  $\text{SO}_2$  radical, and finally, after washing the pulp it is subjected to a further treatment with a relatively small amount of a chlorine agent, 35 preferably ordinary bleaching powder. The improved method is thus carried out in three stages which, when applied to the bleaching of sulphate or "kraft" pulp, are conducted substantially as follows:—

40 *First stage.*—The "kraft" pulp is bleached with the requisite amount of bleaching powder to produce a light yellow color, the amount of bleaching powder being preferably such as to produce the maximum effect 45 without seriously injuring the characteristic strength and toughness of the "kraft" pulp and without materially reducing its yield. This amount of bleaching agent will vary in accordance with the character of the pulp.

Thus, if the stock has been drastically 50 pulped a relatively smaller amount of bleach will be required than for a low cooked or hard pulp. For most commercial purposes an amount of bleach equivalent to from 15 to 30 per cent of bleaching powder containing 55 35 per cent of available chlorine will be employed, such percentage being based upon the weight of the dry stock. Usually, however for a medium cooked stock, the amount of bleaching powder employed in the 60 initial stage will vary from 18 to 23 per cent. The initial bleaching can be effected with any of the different forms of bleacher now used in which the stock density varies 65 from  $4\frac{1}{2}$  to 16 per cent. The temperature employed may vary from ordinary room temperature to 104 degrees F., dependent upon the condition of the bleacher. That is to say, in a high density bleacher no heat 70 would be applied, but where the stock is to be bleached at low density, say  $4\frac{1}{2}$  per cent, heat will be used in order to save time. It is also noted that if sufficient time and the necessary equipment are available, a saving 75 in bleaching powder and a somewhat better result can be produced if this initial bleaching is carried out in two stages, i. e., by adding about three-quarters of the total amount of bleaching agent for the preliminary treatment and after exhaustion of this 80 amount of bleaching powder, washing the pulp and then subjecting it to the remaining quarter of the total amount of bleaching powder employed. This initial stage of the 85 method bleaches the "kraft" pulp from its characteristic brown color to a light yellow and since an excessive amount of bleaching agent is not employed its strength and yield are not materially impaired.

90 *Second stage.*—After exhaustion of the chlorine bleaching agent employed in the first stage, the pulp is treated with from 2 to 5 per cent of sodium bisulphite based on the dry weight of the stock and equivalent to from 40 to 100 pounds per ton of dry pulp. 95 After subjecting the pulp to the action of the sodium bisulphite for about one hour, it is well washed to effect the removal of

the decomposition products and any excess of bisulphite. The bisulphite can be added without washing out the bleach residues from the first stage of the treatment, but slightly better results are attained if these products are first removed by washing. The bisulphite treatment removes the yellow color due to the chlorinated products that are formed in the first stage of the bleaching and which cannot readily be removed by direct treatment with bleaching powder or an equivalent chlorine bleaching agent. Such removal of the color of the chlorinated products is thought to be effected partially by the reduction of such products by the bisulphite and partially by the combination of the bisulphite therewith.

While a suitable sulphite and preferably sodium bisulphite is employed, other reducing agents carrying an  $\text{SO}_2$  radical may be substituted.

*Third stage.*—The stock is now washed and is subjected to a final treatment of a shall amount of the chlorine bleaching agent. Preferably, bleaching powder is employed in the proportion of from 1 to 5 per cent by weight of the original dry stock, that is from 20 to 100 pounds of bleaching powder per ton of dry pulp. Usually about 60 pounds will be found to produce satisfactory results when employing a usual form of bleacher. On exhaustion of the bleaching powder employed in this final stage, the stock is washed and handled in the usual way.

As stated, ordinary sulphate or "kraft" pulp cannot be satisfactorily bleached to produce a white color with a chlorine agent, but by treating the pulp in accordance with the present improved process, first with sufficient bleaching powder to produce a maximum effect without seriously decreasing its yield or strength, and then treating it as described with a substantial amount of sodium bisulphite, it is found that the bisulphite changes the yellow chlorinated coloring compounds produced in the first treatment, probably both by reduction and by direct addition thereto, so that the bulk of these yellow coloring compounds are removed by washing. It is then found that the pulp is in such condition that a very small amount of bleaching powder will bring the final product to a satisfactory white color.

As has been noted, satisfactory commercial results cannot be obtained by methods now generally in use in bleaching sulphate or "kraft" pulp to a white color. Furthermore, even when it is bleached to a very light manila, there is, with the usual methods, a loss in strength of about 30 per cent upwards and a loss in yield of approximately 10 per cent. With the present improved method, it is found that a good white color can be produced, for example with a medium cooked "kraft" pulp, with a loss in

strength of only 8 to 12 per cent and a loss in yield of only about 3 to 5 per cent. Furthermore, there is a very marked saving in the amount of bleaching powder required.

Changes may be made in the details set forth without departure from the essentials of the invention as defined in the claims.

I claim as my invention:

1. The method of bleaching sulphate or kraft pulp to a white color without substantial decrease in the strength or yield, which consists in effecting a partial bleach with an oxidizing bleaching agent, then subjecting the partially bleached pulp to the action of a reducing bleaching agent to reduce and convert the contained coloring compounds, and then effecting a final bleaching action by the use of a relatively small amount of an oxidizing bleaching agent, substantially as described. 75 80 85

2. The method of bleaching chemical wood pulp which consists in subjecting the same to the action of a chlorine bleaching agent, then subjecting the same to the action of a reducing bleaching agent containing an  $\text{SO}_2$  radical and finally to the action of a relatively small amount of a chlorine bleaching agent, substantially as described. 90

3. The method of bleaching sulphate or kraft pulp which consists in subjecting the same to the action of a chlorine bleaching to produce the maximum effect without substantial decrease in strength or yield, and completing the operation by subjecting the partially bleached pulp in successive stages to the action of bleaching agents containing an  $\text{SO}_2$  radical and chlorine respectively. 95 100

4. The method of bleaching chemical pulp which consists in treating the same initially with a hypo-chlorite in amount sufficient to produce a maximum effect without substantial reduction in strength or yield, and then treating the same, in successive stages, with sulphite and chlorine bleaching agents substantially as specified. 105 110

5. The method of producing a white sulphate or kraft pulp which consists in subjecting bleached sulphate pulp successively to the action of sodium bi-sulphite and bleaching powder substantially in the proportions of from 40 to 100 pounds of bi-sulphite and of from 20 to 100 pounds of bleaching powder per ton of dry pulp, substantially as described. 115

6. The method of bleaching sulphate or kraft pulp which consists in treating the same in successive stages, first with from 15 to 25 per cent of bleaching powder, then, with from 2 to 5 per cent of sodium bi-sulphite and finally, with from 1 to 5 per cent of bleaching powder, substantially as described. 120 125

7. The method of bleaching chemical wood pulp which consists in treating the same in 130

successive stages to an oxidizing chlorine bleaching agent and to a reducing bleaching agent containing an  $\text{SO}_2$  radical, then washing the pulp and effecting a final bleach with a relatively small amount of a chlorine bleaching agent, substantially as described.

5. The method of producing a white sul-

phate or kraft pulp which consists in treating the same in successive stages with bleaching powder and sodium bi-sulphite, then washing the same and completing the bleach with a relatively small amount of bleaching powder, substantially as described.

10 OTTO KRESS.